

May 2, 1961

A. M. KAPRAL

2,982,675

METHOD OF WATER-AND GREASE-PROOFING PAPER PRODUCTS

Filed May 8, 1956



## 1

2,982,675

**METHOD OF WATER- AND GREASE-PROOFING PAPER PRODUCTS**

Ales Maria Kapral, Kingsford, near Sydney, New South Wales, Australia, assignor to Process Methods Corporation, Chicago, Ill., a corporation of Illinois

Filed May 8, 1956, Ser. No. 583,479

Claims priority, application Australia May 12, 1955

13 Claims. (Cl. 117—154)

This invention has reference to a method of treating a manufactured paper product, which term is to be taken to include both paper and cardboard, so as to render it resistant to the effects of water and grease.

It is well known that paper can be made impervious to water and grease by treating its surface with water- and grease-repellent or resistant substances. Various methods for the impregnation of paper are known in the art, such methods employing paraffins and/or waxes, or mixtures of paraffins and/or waxes with rubber-latex, resins, rosin, or metallic soaps under various conditions, frequently in the molten state, but sometimes in the form of solutions or emulsions.

These known treating methods have, for instance, the following disadvantages. Comparatively large quantities of wax or the like have to be applied to the paper. Penetration of the substances applied and their adhesion to the surface are not always adequate, so that the coating may peel off and goods wrapped therein are exposed to possible contamination. It may be difficult or even impossible to incorporate into the coat additives such as flavors, insect repellents, preservatives, and the like. The coherent coat closes the pores and prevents passage of air, so that the material to be wrapped cannot breathe.

It is the object of the present invention to avoid these disadvantages and this is achieved according to the invention, inter alia, by the impregnation of manufactured paper and cardboard with a substantially water-insoluble metallic salt of a long-chain carboxylic acid.

According to the invention, printed, colored or plain paper or cardboard is impregnated with a substantially water-insoluble metallic salt or salts of a natural or synthetic long-chain saturated or unsaturated carboxylic acid or acids having a chain length of at least 11 carbon atoms in the molecule, the metal having a valency of at least two and said metallic salt or salts being formed during the impregnation within or on the cellulose fiber of the paper or cardboard, preferably in the presence of ammonia and/or of organic amines.

A machine-unit suitable for water- and grease-proofing manufactured paper and cardboard with a substantially water-insoluble metallic salt of a long-chain carboxylic acid may comprise an endless conveyor belt pervious to liquids and adapted for transporting sheets of paper or cardboard, two or more than two pairs of coating rollers, the rollers of each pair bearing upon said belt from opposite sides, and said pairs of rollers being in spaced relationship to one another for supplying to said paper or cardboard treating solutions being, respectively, a hot aqueous solution of an alkali salt of a long-chain carboxylic acid with or without other additions, and an aqueous solution of an inorganic or organic higher metal salt capable of forming a substantially water-insoluble metallic salt of a long-chain carboxylic acid, the unit further including a heating chamber for drying the paper or cardboard after treatment.

The method of water- and grease-proofing manufac-

## 2

tured paper and cardboard and a specific embodiment of a machine unit for carrying said method into effect are hereinafter described, by way of example only, with reference to the accompanying diagrammatic drawings 5 which show in Fig. 1 the machine unit in side elevation, the method being further illustrated by a number of non-limitative examples, and in Fig. 2 an alternative construction for a part of the machine.

In one embodiment of the method, the paper or cardboard is treated in a first step with a hot or boiling aqueous solution of an alkali metal and/or ammonium salt of such carboxylic acid, and in a second reaction step with an aqueous solution of a metal salt capable of forming with said first-mentioned salt or salts a substantially water-insoluble metal salt of the carboxylic acid, the metal of the salt having a valency of at least two. The aqueous solutions used in the first and second reaction steps may be applied to the paper or cardboard by dipping, roller coating, brushing or spraying.

10 The long chain saturated or unsaturated carboxylic acid may be a synthetic fatty acid or a mixture of synthetic fatty acids having chain lengths of at least 11, obtained by oxidation of natural or synthetic hydrocarbons or by hydrogenation of carbon monoxide. Preferably however, it is a natural carboxylic acid having a chain length from 12 to 20 carbon atoms. Suitable natural fatty acids are for instance, oleic acid, lauric acid, myristic acid, palmitic acid and stearic acid. Suitable 15 alkali salts of these fatty acids are, for instance, sodium oleate, potassium stearate and ammonium stearate either alone or in mixture, but similar alkali salts of these and other fatty acids are also usable in the process.

20

These alkali salts are dissolved in hot or boiling water, or if so desired, the aqueous solution of an alkali salt of a fatty acid may be prepared shortly before use by saponification in heat, of one of the aforementioned fatty acids with an equimolecular or an excess quantity of an alkali hydroxide such as ammonium hydroxide or potassium hydroxide, or of an alkali carbonate, such as sodium carbonate. Saponification may also be effected by, or in the presence of, a suitable organic amine such as triethanolamine.

These alkali salts are dissolved in hot or boiling water, or if so desired, the aqueous solution of an alkali salt of a fatty acid may be prepared shortly before use by saponification in heat, of one of the aforementioned fatty acids with an equimolecular or an excess quantity of an alkali hydroxide such as ammonium hydroxide or potassium hydroxide, or of an alkali carbonate, such as sodium carbonate. Saponification may also be effected by, or in the presence of, a suitable organic amine such as triethanolamine.

25

Tests have shown that it is of particular and unexpected technical advantage to add to the aqueous solution of an alkali salt of said fatty acid or acids a quantity of hexamethylene-tetramine. It has been found that such solution penetrates quicker the minute pores and channels of the cellulose fibers and produces an improved impregnation by some not easily explainable effect on the cellulose of the hexamethylene-tetramine and/or of the free ammonia and free formaldehyde developing therefrom as decomposition products during a subsequent heat-treatment.

If so desired, organic water-soluble dyestuffs may be added to the first solution, or may be applied to the paper after the application of the solution in a separate production step, so as to give the paper a permanent colouring or tint.

Subsequent to such first treatment, the wet paper or cardboard is treated in a second step of the reaction either once or repeatedly with an aqueous solution of an inorganic or organic salt or salts of a metal having a valency of at least two. The fatty acid salts of said metals must be substantially insoluble in water and, if intended for use in connection with foodstuffs, they must be non-toxic and compatible with legislation relating to pure food. Suitable metal salts are, for instance, aluminum sulphate, potassium aluminum sulphate, iron sulphate and aluminum acetate.

The wet alkali salts of long-chain fatty acids applied to the paper react with the metal salts subsequently applied,

within or direct on the cellulose fibers, forming substantially water-insoluble metal salts of fatty acids which are colloidally dispersed in the pores and capillaries of the cellulose fibers, an alkali salt being formed at the same time.

It may be of advantage, at this stage, to remove the alkali salts formed during the reaction by washing, i.e. wetting the paper with water, and subsequent squeezing. However, small quantities of salts may still remain in the pores and, therefore, sulphates and phosphates are preferred for instance to chlorides, as their sodium or potassium salts formed during the reaction are non-hygroscopic.

If ammonia salts of long-chain fatty acids are used in the first reaction step, ammonia being preferably in excess, and the precipitation is brought about in the second reaction step by the use of aluminum acetate, then any danger of salts being hidden in the pores is practically eliminated, because ammonium acetate which may be formed is heat-volatile and acetic acid and ammonia will evaporate as a mixture during the subsequent drying process described hereafter.

After the chemical treatment is completed, the paper or cardboard is dried by passing it through a heating chamber at a temperature of up to about 400 degrees C. The paper may remain in the heating chamber for about 20 seconds to about 2 minutes, depending on the actual drying temperature.

The aforescribed process renders any type of paper water- and grease-resistant, thin paper acquiring the appearance and some of the advantageous properties of a vegetable parchment. However, if cheap grades of paper, such as newsprint are used, such resistance may not be permanent and may decrease over a period of time.

According to a further feature of the invention this disadvantage is overcome and the permanency of the impregnation is considerably improved by treating the paper prior to, during, or after the described chemical reaction with a selected protective colloid, such as alginic acid, a water-soluble salt of alginic acid, gluten, casein and the like. It is preferred however to add the protective colloid to the alkali solution used in the first reaction step.

Alginic acid, its salts, gluten and casein are capable of acting as protective colloids as they envelop the particles of the water-insoluble fatty acid salt and thus act as stabilizers. Therefore, practically permanent water- and grease-resistance of the paper or cardboard is assured by such treatment.

The aforescribed method of water and grease proofing of paper and cardboard, in addition to being economical has the further technical advantage, especially for the production of food wrappers, that certain substances can be added to the solutions, such as a specific perfume or aroma appropriate to the type of product to be wrapped and/or insect repellents, or fungicides, or bactericides, or the like. Thus, for instance, sodium propionate and/or digitalis or like glucosides may be added to the solution.

If, additionally, imperviousness to air is required, it is possible to add to and to disperse in the alkali solution of a fatty acid salt containing ammonia and/or an organic amine used in the first reaction step, small quantities of natural or synthetic rubber latex with or without vulcanizing additives or, alternatively, of a vinyl or of another resin emulsion.

A paper treated according to the aforescribed method is not heat sealing, but a wrapper made thereof can be rendered so by the application of heat sealing compounds such as thermoplastic adhesives, gutta percha and the like to appropriate sections of the wrapper.

A particular advantage of the method of water- and grease-proofing paper and cardboard according to the invention, may be seen in the fact that paper or cardboard so treated will lose its natural smell which in many

instances precludes its use in the food industry. Additionally, after treatment the paper will be practically free of bacteria.

The following non-limitative examples serve to illustrate the method according to this invention, of water- and grease-proofing manufactured paper and cardboard. In each of these examples the hot solution used for the first reaction step is termed solution A for the sake of shortness and the solution used in the 2nd reaction step is, accordingly, termed solution B.

#### Example 1

##### Solution A:

27 gms. stearic acid,  
4.5 gms. potassium hydroxide, and  
9 gms. hexamethylene-tetramine

are added to 1 gallon of boiling water while stirring, and are dissolved. Sheets of paper are treated with the solution A either by dipping them into or by passing them through a bath containing the solution, or by roller coating or, alternatively, by spray application.

Solution B contains 18 gms. of aluminum sulphate per 1 gallon of water. After the first treatment is completed the paper is passed through a cold bath consisting of solution B. Also this second treatment can be carried out in various ways, e.g. by coating the paper by means of rollers covered with rubber or plastic sponge-like material, or by spraying.

Potassium stearate from solution A reacts with the aluminum sulphate from solution B and forms water-insoluble aluminum stearate within, or direct on the cellulose fiber, the hexamethylene-tetramine aids the penetration and improves the impregnation.

The paper is then dried by passing it through a heating chamber. The temperature of the heated air entering the chamber is thermostatically controlled and kept at about 400 degrees C. The paper remains in the chamber for about 65 to 70 seconds. Within the chamber the paper passes through regions of decreasing temperature, so that it can be re-stacked without further precautions immediately after leaving the heating chamber.

#### Example 2

##### Solution A:

27 gms. oleic acid,  
9 gms. sodium carbonate  
9 gms. ammonium hydroxide, and  
4.5 gms. hexamethylene-tetramine

are added to 1 gallon of boiling water, whilst agitating. The paper is treated with the solution A and subsequently with a solution B containing 9 gms. of aluminum potassium sulphate in 1 gallon of cold water. The paper is then dried as described in Example 1.

#### Example 3

##### Solution A:

27 gms. stearic acid and  
4.5 gms. ammonium hydroxide

are dissolved while stirring in 1 gallon of boiling water. If so desired, 9 gms. of hexamethylene-tetramine may be added to solution A. However, this is not necessary, as ammonium hydroxide is considerably in excess and penetration is assured.

The paper is treated with the first solution A and subsequently with a cold solution B containing 9 gms. of freshly prepared aluminum acetate in 1 gallon of water. The paper is then dried as described in Example 1.

#### Example 4

A first solution A is prepared by dissolving under agitation in 1 gallon of boiling water

27 gms. stearic acid,  
9 gms. ammonium carbonate, and  
9 gms. hexamethylene-tetramine

Solution B contains in 1 gallon of cold water 9 gms. ferrous sulphate. The method conforms to that described in Example 1.

*Example 5*

Solution A contains in 1 gallon of boiling water:

27 gms. stearic acid,  
9 gms. triethanolamine,  
18 gms. ammonium hydroxide, and  
9 gms. hexamethylene-tetramine.

Solution B consists of 4.5 gms. of aluminum sulphate and 4.5 gms. of aluminum acetate, in 1 gallon of water.

*Example 6*

Solution A is prepared by dissolving under agitation in 1 gallon of boiling water:

27 gms. stearic acid,  
18 gms. hexamethylene-tetramine, and  
9 gms. ammonium hydroxide.

Solution B consists of 9 gms. of aluminum sulphate in 1 gallon of water.

The method illustrated in any one of Examples 1 to 6 may be modified by the addition to solution A, for the purposes set out above, of any one or more of the following: synthetic or natural rubber latex, polyvinyl or like resin emulsions, flavors, perfumes, bactericides such as digitalis or like glycosides, insecticides, fungicides such as sodium propionate, preservatives, e.g. sodium benzoate or sodium salicylate.

Moreover protective colloids may be added to the ammoniacal fatty acid salt solution in order to increase the permanency of the water and grease-resistance of the paper or the like. It has been found that gluten, casein and alginic acid are particularly suitable protective colloids. Their use is exemplified in the following examples.

*Example 7*

Solution A:

27 gms. oleic acid,  
9 gms. sodium carbonate,  
9 gms. ammonium hydroxide,  
4.5 gms. hexamethylene-tetramine, and  
4.5 gms. gluten.

are added under agitation to 1 gallon of boiling water, and the solution thus obtained is used for the first treatment. The second treatment and the drying are carried out as described in any one of Examples 1 to 6.

*Example 8*

Solution A:

27 gms. stearic acid,  
45 gms. ammonium hydroxide,  
9 gms. gluten, and  
27 gms. synthetic or natural rubber latex

are added under agitation to 1 gallon of boiling water. The colloidal solution A thus obtained is used for the first treatment and the process completed as described in any one of Examples 1 to 6.

*Example 9*

9 gms. of casein are mixed with 27 gms. of water. After standing for about 20 minutes during which time the casein is allowed to swell, the casein paste is added to any one of the solutions A described in Examples 1 to 6.

*Example 10*

4.5 gms. of alginic acid are added to any one of the alkali salt solutions A of fatty acids used for the first treatment according to Examples 1 to 6.

The treatment of paper according to any one of the aforesaid examples leaves the weight of the paper practi-

cally unchanged, the increase of weight being of the order of about 0.01 to 0.1 percent.

The accompanying drawing shows diagrammatically an apparatus suitable for use in carrying out the operations described above. In the drawing,

Fig. 1 is a transverse sectional view of the apparatus assembly for handling paper products to carry out the method of this invention; and

Fig. 2 is a similar view of a modified form of a portion of the apparatus shown in Fig. 1.

The apparatus shown in the drawing substantially comprises an endless conveyor belt 1 which is pervious to liquid, means for feeding or conveying sheets of paper one by one from a stack 2 onto said belt 1, two pairs of coating rollers 3, 4, and 5, 6 in spaced relationship to one another, and a drying chamber 7, the rollers of each of said pairs bearing upon the belt 1 from opposite sides and being associated with a supply for the solutions A and B, respectively, in such a manner that these solutions are applied to both sides of the paper.

The belt 1 is carried by two end rollers 8 and 9, one of which, e.g. roller 8, is a driving roller connected to a prime-mover (not shown). Additionally, the belt 1 is supported between its ends by idling rollers 10, 11 and 12. The belt 1 is made of corrosion-proof wire gauze, wire netting or perforated material. Preferably, the material used for the belt is stainless steel.

The supported ends of the belt are arranged outside the drying chamber 7 which, in the form shown, is provided with additional belts 1A and 1B below belt 1, the paper being transferred from each belt to the belt beneath by optional means, before leaving the chamber 7 in a dried condition.

In operation, sheets of paper are picked up from the stack 2 and are placed on the belt 1 by a suction transfer device 13. On its upper run, and before entering the drying chamber 7, the belt 1 passes the upper rollers 3 and 5 of the two pairs, which bear upon its top and which preferably are each positioned above the lower roller 4 and 6, respectively, which bears upon the lower belt surface. The axes of all rollers 3, 4, 5 and 6 are substantially parallel to one another and to those of the end rollers 8 and 9.

Solution A is supplied to the upper coating roller 3 substantially over its entire length from a suitable receptacle 14. The lower roller 4 receives solution A from a trough 15 wherein it is rotatably supported.

Similarly, solution B is supplied to the upper coating roller 5 substantially over its entire length from a receptacle 16 whereas the lower roller 6 receives solution B from a trough 17.

All coating rollers are preferably positively driven to ensure the greatest possible uniformity of liquid transfer. In the form shown, the upper rollers 3 and 5 each cooperate with a doctor roller 18 and 19 interposed, respectively, between the upper roller and the receptacle above it, the doctor rollers 18, 19 serving to further equalize the quantity and to improve the distribution of liquid transferred to the paper by the rollers 3 and 5. It is of advantage to so arrange the doctor rollers 18 and 19 that they are adjustable with respect to the receptacles 14 and 16, respectively, and/or to the coating rollers 3 and 5, respectively.

The lower coating rollers 4 and 6 also may each be associated with a doctor roller (not shown), if so desired. The troughs 15 and 17 and/or the liquid level therein may be adjustable.

Preferably each pair of coating rollers 3, 4 and 5, 6 is associated with a pair of squeezing rollers 20, 21 and 22, 23 respectively, which bear upon the upper run of the belt 1 from opposite sides and are properly spaced from the coating rollers 3, 4 and 5, 6. The squeezing rollers improve the distribution of liquid within and over the paper and they remove surplus liquid. The

latter may be collected in open troughs 24 and 25 situated below the respective pairs of squeezing rollers.

The belt 1, with the wet paper passes over the supporting and guiding roller 12 into the heating chamber 7. Water sprays 26 and 27 arranged at that station, outside the chamber 7 above and below the belt 1, respectively, serve the purpose of washing away water-soluble alkali salt formed on the sheets during the impregnation.

The heating chamber 7 is of optional size and shape. Air is supplied to it by a blower 28 and it is thermally or electrically heated within a chamber 29 before it enters the chamber 7 through a number of ducts 30, which discharge the hot air below the upper runs of the respective belts 1, 1A and 1B. Appropriate means may be provided for keeping the hot air entering the chamber 7 substantially constant, e.g. at about 400 degrees C.

The wet paper passed through the chamber 7 on the belt 1 is transferred from the latter to the belt 1A beneath it through a chute 31 which preferably accommodates a mechanically operated jockey or equivalent (not shown), and is therefore arranged outside the chamber 7. Similarly, the paper is transferred from the belt 1A to the belt 1B through a chute 32. Finally the paper is discharged from the chamber 7 in dry or substantially dry condition by a suction device 33, and is collected at 34.

For economy, the hot and moist air escaping the top of the chamber 7 through a flue 35 is passed through a condenser 36 from which the condensed water is removed through an outlet 37, while comparatively dry and warm air is returned to the chamber 29 via a down pipe 38 by the suction of the blower or fan 28.

Fig. 2 shows an arrangement in which there is placed in the trough 15 a quartz crystal transducer 39 connected to an oscillator 40 capable of generating ultra-sonic oscillations which are fed to the crystal 39 through the cable 41. An air space 42 is left below the crystal. It has been found that the continuous agitation of the solution by ultra-sonic frequencies leads, particularly when the solution contains ingredients, which are not strictly speaking in solution, to a more even distribution of the components of the solution and thus to a more even distribution of them on the sheets of paper. It has also been found, although the reason for it is not understood, that such agitation leads to a better penetration of the solution into the paper.

I desire it to be understood that I do not wish protection by Letters Patent to be limited to the aforescribed details as these are capable of further modification within the scope of the appended claims.

Thus, for instance, rolls of paper may be treated in a substantially continuous process, instead of treating separate sheets, in a plant resembling, in general, that of printing machinery, but including a section or sections of paper transfer wherein solutions A and B as described above are applied either to one side or to both sides of the paper as it passes said section or sections. If so desired the means for grease-proofing may be associated directly with a printing machine.

What I claim is:

1. A method of water-proofing and grease-proofing paper sheet material comprising the steps of moving said material in a path through the air, directly and positively applying to at least one face of said paper sheet material in a first reaction step a hot aqueous solution of a compound selected from the group consisting of alkali metal salts and ammonium salts of a long chain carboxylic acid having a chain length of at least 11 carbon atoms in the molecule, and in a second reaction step directly and positively applying to said one face of said paper sheet material an aqueous solution of a salt of a metal having a valency of at least 2 and reactive with said first-named compound to form a substantially water-insoluble salt of said carboxylic acid, one of said solutions containing hexamethylenetetramine, whereby said one face of said paper sheet material is impregnated in situ with said substantially water-insoluble salt of said carboxylic acid in the presence of said hexamethylenetetramine in close association with the cellulose fibers at and near said face of said paper sheet material and said paper sheet material is rendered effectively water-proof and grease-proof.

5 2. Method as claimed in claim 1, wherein the long-chain carboxylic acid is selected from the group of natural fatty acids consisting of oleic acid, lauric acid, myristic acid, palmitic acid and stearic acid.

3. Method as claimed in claim 1, wherein the substantially water-insoluble metallic salt of a carboxylic acid is formed in the presence of triethanolamine.

4. Method as claimed in claim 1, wherein the water-insoluble metallic salt is an aluminum salt.

5. Method as claimed in claim 1, wherein the water-insoluble metallic salt is an iron salt.

6. Method as claimed in claim 1, wherein the metallic salt capable of forming a substantially water-insoluble metallic salt of a carboxylic acid, used in the second reaction step is selected from the group of salts consisting of phosphates, sulphates and acetates.

7. Method as claimed in claim 1, wherein a protective colloid is added to the aqueous solution used in the first reaction step.

8. Method as claimed in claim 7, wherein the protective colloid is selected from the group consisting of gluten, alginic acid, water-soluble salts of alginic acid and casein.

9. Method as claimed in claim 1, wherein a polyvinyl resin emulsion is added to the aqueous solution used in the first reaction step.

10. Method as claimed in claim 1, wherein a material selected from the group consisting of sodium propionate and glycosides is added to the aqueous solution used in the first reaction step.

11. Method as claimed in claim 1, wherein in the first reaction step the said aqueous solution is agitated by means of ultra-sonic vibrations.

12. A water-proof and grease-proof paper sheet produced by moving said material in a path through the air, directly and positively applying to at least one face of said paper sheet material in a first reaction step a hot aqueous solution of a compound selected from the group consisting of alkali metal salts and ammonium salts of a long chain carboxylic acid having a chain length of at least 11 carbon atoms in the molecule, and in a second reaction step directly and positively applying to said one face of said paper sheet material an aqueous solution of a salt of a metal having a valency of at least 2 and reactive with said first-named compound to form a substantially water-insoluble salt of said carboxylic acid, one of said solutions containing hexamethylenetetramine, whereby said one face of said paper sheet material is impregnated in situ with said substantially water-insoluble salt of said carboxylic acid in the presence of said hexamethylenetetramine, in close association with the cellulose fibers at and near said face of said paper sheet material and said paper sheet material is rendered effectively water-proof and grease-proof.

13. A water-proof and grease-proof paper sheet produced by moving said material in a path through the air, directly and positively applying to at least one face of said paper sheet material in a first reaction step a hot aqueous solution of a compound selected from the group consisting of alkali metal salts and ammonium salts of a long chain carboxylic acid having a chain length of at least 11 carbon atoms in the molecule and selected from the group consisting of oleic acid, myristic acid, palmitic acid and stearic acid, and in a second reaction step directly and positively applying to said one face of said paper sheet material an aqueous solution of a salt of a metal having a valency of at least 2 and reactive with said first-named compound to form a substantially water-insoluble salt of said carboxylic acid, one of said solutions containing hexamethylenetetramine, whereby said one face of said paper sheet material is impregnated in situ with said substantially water-insoluble salt of said carboxylic acid in the presence of said hexamethylenetetramine, in close association with the cellulose fibers at and near said face of said paper sheet material and said paper sheet material is rendered effectively water-proof and grease-proof.

ing a valency of at least 2 selected from the group consisting of phosphates, sulphates and acetates and reactive with said first-named compound to form a substantially water-insoluble salt of said carboxylic acid, one of said solutions containing hexamethylenetetramine whereby said one face of said paper sheet material is impregnated in situ with said substantially water-insoluble salt of said carboxylic acid in the presence of said hexamethylenetetramine in close association with the cellulose fibers at and near said face of said paper sheet material and 10 said paper sheet material is rendered effectively waterproof and grease-proof.

## References Cited in the file of this patent

## UNITED STATES PATENTS

15

|           |               |               |
|-----------|---------------|---------------|
| 742,212   | Muller-Jacobs | Oct. 27, 1903 |
| 1,270,055 | Richards      | June 18, 1918 |

|             |                |               |
|-------------|----------------|---------------|
| 1,430,998   | Hoskins        | Oct. 3, 1922  |
| 1,519,803   | Sellows et al. | Dec. 16, 1924 |
| 1,746,648   | Grunbaum       | Feb. 11, 1930 |
| 1,829,877   | Schroeder      | Nov. 3, 1931  |
| 5 1,963,975 | Ellis          | June 26, 1934 |
| 1,982,018   | Owen           | Nov. 27, 1934 |
| 2,021,172   | Bucy           | Nov. 19, 1935 |
| 2,287,348   | Hayden         | June 23, 1942 |
| 2,306,576   | Warth et al.   | Dec. 29, 1942 |
| 2,534,008   | Fiero et al.   | Dec. 12, 1950 |
| 2,603,576   | Cook et al.    | July 15, 1952 |
| 2,635,055   | Figdor         | Apr. 14, 1953 |
| 2,637,535   | Arnold         | May 5, 1953   |
| 2,704,732   | Copeman et al. | Mar. 22, 1955 |

## FOREIGN PATENTS

|         |               |             |
|---------|---------------|-------------|
| 536,062 | Great Britain | May 1, 1941 |
|---------|---------------|-------------|